

Feb. 26, 1963

R. K. VAN POUCKE ET AL  
SILVER HALIDE EMULSION CONTAINING  
N-(ALKYLSULFONYLPHENYL)-1-HYDROXY-  
2-NAPHTHOIC ACID AMIDE  
COLOR COUPLERS  
Filed Nov. 3, 1960

3,079,256



P. K. Van Poucke  
P. H. De Cat  
M. H. Verbrugghe,  
BY Watson, Cole, Grindle & Watson

ATTORNEYS

# United States Patent Office

3,079,256

Patented Feb. 26, 1963

1

3,079,256

## SILVER HALIDE EMULSION CONTAINING N.(ALKYLSULFONYLPHENYL)-1-HYDROXY-2-NAPHTHOIC ACID AMIDE COLOR COUPLERS

Raphael Karel Van Poucke, Mechlin, Arthur Henri De Cat, Mortsel-Antwerp, and Marcel Hendrik Verbrughe, Wilrijk-Antwerp, Belgium, assignors to Gevaert Photo-Producten N.V., Mortsel-Antwerp, Belgium, a Belgian company

Filed Nov. 3, 1960, Ser. No. 66,964

Claims priority, application Belgium Nov. 20, 1959  
10 Claims. (Cl. 96—55)

The present invention relates to a process for the manufacture of photographic color images and also to color correction.

It is known that a colored image may be formed by incorporating into the silver halide emulsion a compound which couples during development with the oxidation product of the developing agent and forms a colored compound in the same area where the silver halide grains are reduced.

Such a compound which is employed in conjunction with the developing agent for the silver and which couples with the oxidation product of the developing agent during development is referred to herein as a color-forming compound or coupler.

The modern processes of color photography are based upon the subtractive color principle according to which differently sensitized silver halide emulsions are superposed in the form of layers. Each of these layers contains the different color forming compounds which produce on development the subtractive yellow-cyan- and magenta-color images. The usual developing substance is a primary aromatic amine.

The dyestuffs and pigments used in practice in subtractive processes of color photography do not possess ideal spectral absorption curves. In addition to absorbing light in the desired part of the spectrum, they also absorb some light in other parts of the spectrum and, as a result thereof, the color reproduction is never ideal. For example, cyan dyestuffs formed by color development from color formers of the 1-naphthol series absorb the desired complementary colored red-light and in addition absorb undesirably a certain amount of blue and green light.

It has been proposed to correct for these deficiencies by the use of an automatic masking method, whereby after the usual color development and treatment in a bleaching bath the unchanged color former reacts with the oxidation product of a 4-amino-3-pyrazolone derivative to form a magenta dyestuff so that it absorbs blue and green light at an intensity equal to the undesired blue and green absorption of the cyan dyestuff formed by color development. This process of masking is described in the U.S. application Serial No. 705,508, filed December 27, 1957.

It is known that different demands are made upon the color couplers according to whether they are designed for negative or for positive material. E.g. it is known that 1-hydroxy-2-naphthamide color couplers, giving after color development pure blue images, are preferably used for the manufacture of positive color materials. On the other hand it is preferable for the manufacture of negative materials to use 1-hydroxy-2-naphthamide color couplers producing a cyan image, and the absorption spectrum of which is shifted as far as possible to the longer wave-lengths showing thereby side-absorptions which are as low as possible. But the disadvantage of the bathochromic shifting of the absorption spectrum is that this action in most cases is accompanied by an increase of

2

unwanted side-absorption resp. in the green and blue parts of the spectrum.

To overcome this disadvantage there is a permanent research for cyan color couplers with a bathochromically shifted absorption spectrum whereby, however, the side-absorptions are kept as low as possible in the blue and the green. In connection therewith we refer to the 1-hydroxy-2-naphthoic acid amide color couplers which are manufactured according to the Belgian Patent 548,880.

Now it has been found that it is possible to obtain cyan colored images with increased transparency in the green by using 1-hydroxy-2-naphthoic acid amide color couplers which correspond to the general formula:

15



or

25



30 wherein:

X is a member selected from the group consisting of a hydrogen atom, a halogen atom, a sulphonate acid group or a sulphonate group;

35 Y is a member selected from the group consisting of a hydrogen atom, a carboxyl group, a sulphonate acid group or a sulphonate group;

R represents a radical comprising a linear chain of at least 5 and at most 20 C-atoms making the molecule 40 non-migratory in the emulsion layer.

Comparative absorption curves are given hereinafter which elucidate the favorable absorption spectrum and particularly the increased transparency in the green of 45 the dyestuff images obtained with these color couplers.

An advantage of the color couplers according to the present invention with regards to the above-mentioned U.S. application Serial No. 705,508, filed December 27, 1957, and to the German patent application G 30,580 50 consists therein that they form a mask dyestuff image since they easily react in an oxidative medium with 4-aminopyrazolone-3 and derivatives thereof with the following general formula:

55



60 wherein:

R<sub>1</sub> is a lower alkyl group, e.g. a methyl group;

R<sub>2</sub> represents a lower alkyl group, e.g. a methyl group or an aryl group, such as a phenyl group or a substituted phenyl group;

65 R<sub>3</sub> represents an aliphatic radical making the molecule non-migratory with more than 5 and less than 20 carbon atoms e.g. consisting of a nonyl, an undecyl, a tridecyl or a pentadecyl group.

Examples of such 4-aminopyrazolone-3 are among 70 others:

1,2-dimethyl-4-amino-5-nonylpyrazolone-3

- 1,2-dimethyl-4-amino-5-undecylpyrazolone-3  
 1,2-dimethyl-4-amino-5-tridecylpyrazolone-3  
 1,2-dimethyl-4-amino-5-pentadecylpyrazolone-3  
 1-methyl-2-(p-carbethoxyphenyl)-4-amino-5-pentadecylpyrazolone-3  
 Methyl ester of 1-methyl-2-(p-succinylamidophenyl)-4-amino-5-pentadecylpyrazolone-3  
 1-methyl-2-(2'-chloro-5'-carbomethoxyphenyl)-4-amino-5-pentadecylpyrazolone-3.

The preparation and the use of these compounds is described in the German patent application G 30,580. In this way, the application of the present invention may be possible not only to compensate the remaining low side-absorption in the green but also almost completely the side-absorption in the blue, so that finally a cyan image is obtained the absorption of which is almost ideal.

The new color couplers can be prepared by condensation of a 1-hydroxy-2-naphthoic acid or a derivative thereof with desired aromatic amines. In order to prepare color couplers which contain in their naphthol or anilide group a sulphonate acid group it is advantageous before the condensation to introduce a sulfo-fluoride group into the naphthol resp. anilide group which after condensation is saponified to the corresponding sulphonate acid, e.g. by application of the process described in the Belgian Patents 584,152 and 590,934.

The preparation of such new color couplers is described hereinafter by way of example.

I. Preparation of *N*-(3'-carboxy-4'-cetylphenoxyphenyl)-1-hydroxy-2-naphthoic acid amide.—20 g. of 2-chloro-5-nitrobenzoic acid (Hubner: Ann. 222, 195) are dissolved in 100 cm.<sup>3</sup> of methyl Cellosolve to which 5.6 g. of potassium hydroxide were added. A second solution is obtained by dissolving in 50 cm.<sup>3</sup> of methyl Cellosolve, 25.8 g. of cetyl mercaptane together with 5.6 g. of potassium hydroxide. Both solutions are mixed and refluxed for 1 hour. The potassium chloride obtained is filtrated off, the mixture still being warm. After acidifying with acetic acid and after diluting with 500 cm.<sup>3</sup> of methanol a precipitate is obtained which is recrystallized from methanol. The obtained 2-cetyl-mercapto-5-nitro benzoic acid has a melting point of 108° C.

42.3 g. of this 2-cetylmercapto-5-nitrobenzoic acid are refluxed together with 150 cm.<sup>3</sup> of acetic acid. A dark brown solution is obtained to which 70 cm.<sup>3</sup> of a hydrogen peroxide solution 30% in water are dropwise added whilst stirring (exothermic reaction); refluxing is continued for 1 hour. After cooling a white amorphous product is obtained which is recrystallized from acetic acid giving thereby the 2-cetyl sulphonyl-5-nitrobenzoic acid. Melting point: 97° C.

45.5 g. of this nitrobenzoic acid derivatives which are dissolved in 300 cm.<sup>3</sup> of ethanol are introduced into a hydrogenation autoclave under addition of Raney nickel. Hydrogen is introduced till a pressure of 70 kg./cm.<sup>2</sup> is reached. The temperature is brought at 55° C. Within the course of 3½ hours of shaking the theoretically determined quantity of hydrogen is absorbed. The Raney nickel is filtrated off and the filtrate is evaporated to dryness. After recrystallization from a mixture of acetic acid and water a 2-cetyl sulphonyl-5-aminobenzoic acid is obtained under the form of a white crystalline product. Melting point: 119° C.

12.75 g. of this amino derivative and 7.92 g. of hydroxynaphthoic acid phenyl ester are melted together. The phenol is distilled off under reduced pressure varying between 2 and 5 mm. Hg. The product is poured out into methanol and recrystallized from acetonitrile. White crystals of *N*-(3'-carboxy-4'-cetylphenoxyphenyl)-1-hydroxy-2-naphthoic acid amide are formed in this way. Melting point 146° C.

II. Preparation of *N*-(o-cetylphenoxyphenyl)-1-hydroxy-4-chloro-2-naphthoic acid amide.—10.65 g. of 1-hydroxy-4-chloro-2-phenyl naphthoate (J. Univ. Bombay

(NS) 10 part 5, Sect. A, pp. 131-134) and 13.64 g. of o-cetylphenoxyphenyl are before thoroughly mixing heated to 170° C. on an oil-bath. The phenol is distilled off under a reduced pressure of ±8 mm. After 2 hours the heated reaction mixture is poured out into methanol. After recrystallization from a mixture of benzene and hexane a granular product is obtained. Melting point: 102° C.

III. The preparation of *N*-(6'-cetylphenoxyphenyl)-1-hydroxy-2-naphthoic acid amide-3'-sodium sulphonate is described in the German patent application G 30,287 (preparation 13).

IV. Preparation of *N*-(6'-cetylphenoxyphenyl)-1-hydroxy-4-chloro-2-naphthoic acid amide-3'-sodium sulphonate is described in German patent application G 30,287 (preparation 15).

V. Preparation of *N*-(6'-cetylphenoxyphenyl)-1-hydroxy-2-naphthoic acid amide-3'-4-disodium sulphonate is described in the German patent application G 30,287 (preparation 16).

VI. Preparation of *N*-(4'-cetylphenoxyphenyl)-1-hydroxy-2-naphthoic acid amide-3'-sodium sulphonate is described in the German patent application G 30,287 (preparation 14).

VII. The preparation of *N*-(o-cetylphenoxyphenyl)-1-hydroxy-2-naphthoic acid amide-4-sodium sulphonate is described in Belgian patent specification 584,152—Table II, Example 5.

For carrying out the process according to the present invention, the color couplers and mask compounds must be incorporated into a photographic silver halide emulsion prepared by means of the usual colloids, such as for instance gelatin, polyvinyl alcohol, colloidion or other natural or synthetic colloids and such as for instance those of the Belgian Patent 568,153. The silver halide emulsion can be coated on a support consisting of paper, glass, nitrocellulose, cellulose esters such as cellulose triacetate, polyester, polystyrene or another natural or synthetic resin, and form part of a photographic material with one or more emulsion layers. The multilayer material is usually composed of the following sequence of layers: a support, an emulsion layer sensitized to red having a color coupler for cyan, an emulsion layer sensitized to green having a color coupler for magenta and an emulsion layer sensitive to blue having a color coupler for yellow. There is a yellow filter composed in most of the cases of colloidal silver, located between the blue-sensitive and the emulsion layer sensitized to green.

It is not only possible to incorporate the new color couplers into the light-sensitive silver halide emulsion layer itself but they can also be incorporated into an adjacent non-light-sensitive colloid layer or into a non-light-sensitive layer which is separated from the light-sensitive emulsion layer by a water-permeable colloid layer.

The following aromatic amino-compounds can be used as developers for such material: mono-, di- and triaminoaryl compounds, more specifically *N,N*-dialkyl-p-phenylenediamine and its derivatives such as *N,N*-dialkyl-*N'*-sulphomethyl- or carboxy-methyl-p-phenylene diamine. As useful monoamino-developers should be cited: amino-phenols and amino cresols or their halogen derivatives and also the aminonaphthols.

The following examples illustrate the present invention without limiting, however, the scope thereof. We draw the attention to the fact that all the quantities mentioned hereinafter are parts by weight when no other indication is given.

#### EXAMPLE 1

10 parts of *N*-(4'-cetylphenoxyphenyl)-1-hydroxy-2-naphthoic acid amide-3'-sodium sulphonate are wetted by 40 parts of ethanol and brought into solution by heating at 40° C. by means of 20 parts of water. This solution is diluted with water up to 200 parts whereby a solution 5% is obtained. 200 parts of this color coupler solution together with 260 parts of water are added to 500 parts

of a silver bromo-iodide gelatin emulsion (2% iodide). The usual solutions which contain hardening and wetting agents are added to the emulsion. The resulting emulsion is coated on a suitable support. The photographic material which is obtained after drying, is exposed and afterwards submitted to color development in a bath of the following composition:

|                                              |      |    |
|----------------------------------------------|------|----|
| N,N-diethyl-p-phenylenediamine hydrochloride | 2.75 | G. |
| Sodium sulphite                              | 2    | 10 |
| Potassium carbonate                          | 75   |    |
| Potassium bromide                            | 0.5  |    |
| Hydroxylamine hydrochloride                  | 1.2  |    |
| Sodium hexametaphosphate                     | 1.0  |    |
| Water to 1000 cm. <sup>3</sup>               |      |    |

This material is rinsed for 30 seconds and fixed in an acid fixing bath of the following composition:

|                                |     |    |
|--------------------------------|-----|----|
| Sodium thiosulphate (dry)      | 200 | G. |
| Borax                          | 8   | 20 |
| Sodium sulphite                | 25  |    |
| Potassium alum                 | 15  |    |
| Boric acid                     | 7.5 |    |
| Water to 1000 cm. <sup>3</sup> |     |    |

Now the material is rinsed for 10 min. and bleached in a bath of the following composition:

|                                |     |    |
|--------------------------------|-----|----|
| Potassium ferricyanide         | 100 | G. |
| Potassium bromide              | 25  | 30 |
| Borax                          | 20  |    |
| Boric acid                     | 5   |    |
| Water to 1000 cm. <sup>3</sup> |     |    |

Finally the material is rinsed for 5 min. and fixed in a bath of the following composition:

|                                |     |    |
|--------------------------------|-----|----|
| Sodium thiosulphate (dry)      | 130 | G. |
| Sodium sulphite                | 10  |    |
| Sodium carbonate               | 14  |    |
| Water to 1000 cm. <sup>3</sup> |     |    |

An intense cyan image showing very low side-absorptions in the green spectrum is obtained.

#### EXAMPLE 2

10 parts of N-(6'-cetysulphonylphenyl)-1-hydroxy-2-naphthoic acid amide-4,3'-disodium sulphonate are wetted with 20 parts of ethanol and dissolved in 180 parts of water. The color coupler solution is incorporated into the emulsion according to the method described in Example 1. After exposure of the material and further treatment as described in Example 1, a cyan image which shows a very low side absorption in the green and the blue is obtained.

#### EXAMPLE 3

10 parts of N-(3'-carboxy-4'-cetysulphonylphenyl)-1-hydroxy-2-naphthoic acid amide are wetted with 30 parts of ethanol and dissolved in 25 parts of alkali N and 145 parts of water. The color coupler solution is incorporated into the emulsion according to Example 1. The emulsion is neutralized by 7.5 parts of acetic acid N/2 per 100 parts of color coupler solution. The exposure as well as the development are carried out as described in Example 1, taking into account, however, that in the color developing bath the N,N-diethyl-p-phenylene diamine hydrochloride is replaced by 4-amino-N - ethyl - N-( $\beta$ -methyl-sulphonamidoethyl)m-toluidine-sesquisulphate monohydrate. A cyan image with low side absorptions is obtained.

#### EXAMPLE 4

200 parts of a solution 5% of N-(6'-cetysulphonylphenyl)-1-hydroxy-2-naphthoic acid amide-3'-sodium sulphonate dissolved in a mixture of ethanol and water (3:7) and 260 parts of water are added to 500 parts of

5 a red-sensitized silver iodo-bromide-emulsion (2% iodide). This emulsion is coated on a photographic support. After exposure, color development and further treatment according to Example 1, an intense cyan image with low side-absorptions in the green is obtained.

#### EXAMPLE 5

To 450 g. of silver bromo-iodide emulsion and 45 cm.<sup>3</sup> of water are added 20 cm.<sup>3</sup> of a solution 0.1% of the sensitizer for red [2-(3-methyl-5-phenyl-2,3-benzothiazoline)] - [2'-(1' - methylnaphtho[1,2]thiazole)]- $\beta$ -ethyl trimethinecyanine-methylsulphate. To this emulsion are added 70 cm.<sup>3</sup> of an alkaline solution 10% (0.5% sodium hydroxide) of the color coupler for cyan N-(6'-cetysulphonylphenyl)-1-hydroxy-2-naphthoic acid amide-3'-sodium sulphonate together with 25 cm.<sup>3</sup> of an alkaline solution 20% (0.6% sodium hydroxide) of 1,2-dimethyl-4-amino-5-nonyl pyrazolone-3 - hydrochloride. The whole mixture is neutralized by 12 cm.<sup>3</sup> of acetic acid N. This product is as usual chrome hardened whereafter a stabilizing agent together with a wetting agent are added. This emulsion is coated in ratio of 100 g./sq. m. on a photographic support. After exposure, the photographic material thus obtained is treated according to Example 1. Besides a negative cyan image a positive magenta image is formed which compensates completely the unwanted absorptions in the green and to a great extent in the blue.

#### EXAMPLE 6

To a red-sensitized silver bromo-iodide emulsion containing about  $\frac{1}{3}$  mol of silver halide per kg. of emulsion are added per mol of silver halide 240 cm.<sup>3</sup> of a solution 10% of N-(6'-cetysulphonylphenyl)-1-hydroxy-2-naphthoic acid amide-3'-sodium sulphonate in alcohol with a little sodium hydroxide and next 120 cm.<sup>3</sup> of a solution 10% of 1,2 - dimethyl - 4 - amino-5-tridecyl-pyrazolone-3 in methylcellosolve with a little sodium hydroxide. After acidification to pH 6 and after addition of the usual additives such as hardeners, wetting agents and stabilizers, the emulsion obtained is coated on a suitable support and dried. After exposure through a red filter (Gevaafilter R 678 marketed by Gevaert Photo-Producten N.V., Mortsel, Belgium) and a grey wedge with a constant 0.15, the photographic material composed in this way is developed for 9 minutes at 20° C. in a color developing bath with the following composition:

|                                              |     |    |
|----------------------------------------------|-----|----|
| Sodium hexametaphosphate                     | 2   | G. |
| N,N-diethyl-p-phenylenediamine hydrochloride | 3   |    |
| Sodium sulphite                              | 4   |    |
| Sodium carbonate                             | 57  |    |
| Hydroxylamine hydrochloride                  | 1.5 |    |
| Potassium bromide                            | 1   |    |
| Water to 1000 cm. <sup>3</sup> (pH=10.6)     |     |    |

This material is rinsed for 30 minutes at 18 to 20° C. and fixed for 5 minutes at 20° C. in a fixing bath of the following composition:

|                                         |     |    |
|-----------------------------------------|-----|----|
| Sodium thiosulphate                     | 200 | G. |
| Sodium bisulphite                       | 25  |    |
| Potassium alum                          | 20  |    |
| Sodium biacetate                        | 20  |    |
| Boric acid                              | 7.5 |    |
| Water to 1000 cm. <sup>3</sup> (pH=4.0) |     |    |

Next, the material is rinsed again for 10 minutes at 18 to 20° C. and treated for 5 minutes in a bleaching bath of the following composition:

|                                         |     |    |
|-----------------------------------------|-----|----|
| Potassium ferricyanide                  | 100 | G. |
| Potassium bromide                       | 15  |    |
| Borax                                   | 20  |    |
| Magnesium sulphate                      | 50  |    |
| Water to 1000 cm. <sup>3</sup> (pH=8.6) |     |    |

Rinsing is continued for another 10 minutes at 18 to 20° C. and then the material is fixed again for 5 minutes at 20° C. in a bath of the following composition:

|                                          | G.  |
|------------------------------------------|-----|
| Sodium thiosulphate                      | 130 |
| Borax                                    | 20  |
| Magnesium sulphate                       | 50  |
| Water to 1000 cm. <sup>3</sup> (pH=8.9). |     |

Finally, rinsing is continued for 10 minutes at 18 to 20° C. and the material is dried.

After this treatment a cyan image wherein the disturbing influence of the side-absorption is reduced by the formed magenta masking image with opposite gradation to the cyan image obtained.

#### EXAMPLE 7

To a red-sensitized silver bromo-iodide emulsion containing about  $\frac{1}{3}$  mol of silver halide per kg. of emulsion are added per mol of silver halide 240 cm.<sup>3</sup> of a solution 10% of N-(6'-cetyl sulphophenyl)-1-hydroxy-2-naphthoic acid amide-3'-sodium sulphonate in alcohol with a little sodium hydroxide and next 120 cm.<sup>3</sup> of a solution 10% in methylcellosolve of the methylester of 1 - methyl - 2 - (p - succinylamidophenyl)-4-amino-5-pentadecylpyrazolone-3 with a little sodium hydroxide. After further treatment as in Example 6, a cyan image is obtained wherein the disturbing influence of the side-absorptions is reduced by the formed magenta masking image with opposite gradation to the cyan image.

#### EXAMPLE 8

To a red-sensitized silver bromo-iodide emulsion containing about  $\frac{1}{3}$  mol of silver halide per kg. of emulsion are added per mol of silver halide 240 cm.<sup>3</sup> of a solution 10% of N-(6'-cetyl sulphophenyl)-1-hydroxy-2-naphthoic acid amide-3'-sodium sulphonate in alcohol with a little sodium hydroxide and next 120 cm.<sup>3</sup> of a solution 10% in methyl cellosolve of 1-methyl-2-(2'-chloro-5'-carbomethoxyphenyl - 4 - amino-5-pentadecylpyrazolone-3 with a little sodium hydroxide. After further treatment as in Example 6 a cyan image is obtained wherein the disturbing influence of the side-absorption is reduced by the formed magenta mask image with opposite gradation to the cyan image.

#### EXAMPLE 9

Before coating a red-sensitized silver halide emulsion containing  $\frac{1}{3}$  mol of silver halide/kg. emulsion 240 cm.<sup>3</sup> of an alcoholic sodium hydroxide solution 10% of N-(6'-cetyl sulphophenyl)-1-hydroxy-4-chloro - 2 - naphthoic acid amide-3'-sodium sulphonate are added to this emulsion per mol of silver halide and next 120 cm.<sup>3</sup> of a solution 10% of 1,2-dimethyl-4-amino-5-tridecyl-pyrazolone-3 in methyl cellosolve with a little sodium hydroxide.

After acidification with acetic acid to a pH 6 and after the ordinary addition of hardening agents and stabilizers, this emulsion is coated on a support provided with an anti-halation layer. To this emulsion layer is successively coated a thin gelatin layer, a green light-sensitized silver bromo-iodide emulsion layer with a color coupler for magenta, a yellow filter layer consisting of gelatin with dispersed colloidal silver, a blue sensitive silver bromo-iodide silver layer with color coupler for yellow, and finally an anti-stress layer. After exposure and further finishing such as in Example 6, a dyestuff image is obtained the red light-sensitized emulsion layer of which contains a cyan dyestuff image the unfavorable side-absorptions of which are masked by a magenta mask image with opposite gradation.

The accompanying absorption curves give a comparative image of the absorption spectra of compounds prepared before and those prepared according to the present invention.

Curve I: Absorption curve of the developed color coupler prepared according to German patent specifi-

tion 930,795, page 2, lines 34-41 but C<sub>16</sub>H<sub>33</sub> is substituted for C<sub>18</sub>H<sub>37</sub>.

Curve II: Absorption curve of the developed color coupler prepared according to the German specification 1,036,053, Example 1.

Curve III: Absorption curve of the developed color coupler according to preparation III in the foregoing description



The developer for the three cases is N,N-diethyl-p-phenylenediamine.

As appears from the above, the course of curves I and II corresponds somewhat whereas curve III points to a higher transparency in the green of the spectrum.

We claim:

1. Process for obtaining a colored photographic image in a reducible silver halide emulsion layer, comprising exposing said layer and developing same with a primary aromatic amino developing agent in the presence of a color coupler for cyan, selected from the group consisting of



and



wherein

X represents a member selected from the group consisting of a hydrogen atom, a halogen atom, a sulphonate group;

Y represents a member selected from the group consisting of a carboxyl group, a sulphonate group and a sulphonate group.

R represents an aliphatic radical comprising a linear chain of at least 5 and at most 20 C-atoms and rendering said coupler resistant to diffusion:

2. A multilayer photographic color film comprising a plurality of superposed differentially light-sensitive silver halide emulsion layers containing in the red sensitive silver halide emulsion layer a color coupler for cyan selected from the group consisting of



and



wherein

X represents a member selected from the group consisting of a hydrogen atom, a halogen atom, a sulphonic acid group and a sulphonate group;

Y represents a member selected from the group consisting of a carboxyl group, a sulphonate acid group and a sulphonate group;

R represents an aliphatic radical comprising a linear chain of at least 5 and at most 20 C-atoms and rendering said coupler resistant to diffusion.

3. Photographic element having superposed silver halide emulsion layers sensitive to different regions of the visible spectrum, at least one of said layers containing a color coupler for color development selected from the group consisting of:



and



wherein

X represents a member selected from the group consisting of a hydrogen atom, a halogen atom, a sulphonate group and a sulphonate group;

Y represents a member selected from the group consisting of a carboxyl group, a sulphonate group and a sulphonic acid group;

R represents an aliphatic radical comprising a linear chain of at least 5 and at most 20 C-atoms and rendering said coupler resistant to diffusion,

which is reactive with the oxidation product of an aromatic amino developing agent to form by color development a cyan dye image which absorbs a major proportion of light in the red region of the visible spectrum, and undesirably absorbs a minor proportion of light in the

10

at least one other region of the visible spectrum, and a 4-aminopyrazolone-3 derivative with the following general formula



wherein

- 10  $R_1$  represents a member selected from the group consisting of a lower alkyl radical,

15  $R_2$  represents a member selected from the group consisting of a lower alkyl radical and a monocyclic aryl radical of the benzene series,

20  $R_3$  represents an aliphatic radical of more than 5 and less than 20 carbon atoms rendering said derivative resistant to diffusion,

25 said color coupler being also reactive with the oxidation product of said 4-amino-pyrazolone-3 derivative to form a secondary dye image having a graduation opposite to that of said cyan dye image, and absorbing light in at least one of said said unwanted minor absorption regions but transmitting substantially all the light in said major absorption region.

30 4. The photographic element of claim 3 wherein said color coupler is  $N-(4'-cetyl-sulphonylphenyl)-1-hydroxy-2-naphthoic acid amide-3'-sodium sulphonate.$

35 5. The photographic element of claim 3 wherein said color coupler is  $N-(6'-cetyl-sulphonylphenyl)-1-hydroxy-2-naphthoic acid amide-4,3'-disodium sulphonate.$

40 6. The photographic element of claim 3 wherein said color coupler is  $N-(6'-cetyl-sulphonylphenyl)-1-hydroxy-2-naphthoic acid amide-3'-sodium sulphonate.$

45 7. The photographic element of claim 3 wherein said pyrazolone derivative is  $1,2\text{-dimethyl-1,4-amino-5-nonyl-pyrazolone-3-hydrochloride.}$

8. The photographic element of claim 3 wherein said pyrazolone derivative is  $1,2\text{-dimethyl-4-amino-5-tridecyl-pyrazolone-3.}$

9. The photographic element of claim 3 wherein said pyrazolone derivative is  $1\text{-methyl-2-(p-succinylamido-phenyl)-4-amino-5-pentadecylpyrazolone-3.}$

10. The photographic element of claim 3 wherein said pyrazolone derivative is  $1\text{-methyl-2-(2-chloro-5'-carbo-methoxyphenyl)-4-amino-5-pentadecylpyrazolone-3.}$

No references cited.